# EUROPEAN PATENT SPECIFICATION

(11) **EP 0 655 033 B1**
(45) Date of publication and mention of the grant of the patent: **11.12.1996**
(21) Application number: 92917131.2
(22) Date of filing: 12.08.1992
(51) Int. Cl.: B41M 5/26, B41M 5/38

(54) **THERMAL TRANSFER IMAGING**
BILDÜBERTRAGUNGSVERFAHREN DURCH WÄRME
IMAGERIE PAR TRANSFERT THERMIQUE

(43) Date of publication of application: 31.05.1995
(73) Proprietor: MINNESOTA MINING AND MANUFACTURING COMPANY, St. Paul, Minnesota 55133-3427 (US)
(72) Inventor: PATEL, Ranjan Chhaganbhai George Green Cottage, Essex CM22 7PP (GB); CHOU, Hsin-Hsin, Woodbury, NM 55125 (US); KAM, Keung Kam, Woodbury, MN 55125 (US)
(74) Representative: Bowman, Paul Alan
(86) International application number: GB9201489
(87) International publication number: WO9404368

(56) References cited:
- JP-A- 4 153 087
- US-A- 4 587 198
- US-A- 5 139 598

## Description

The present invention relates to a method of thermal transfer imaging, in which a scanning exposure source, such as a laser, is used to effect the thermal transfer of colourant from a donor sheet to a receptor for the thermally transferred colourant.

Thermal transfer imaging involves the imagewise transfer of colourant from a donor sheet to a receptor sheet under the action of heat, the donor and receptor sheets being maintained in intimate, face-to-face contact throughout. This type of imaging is increasingly popular, mainly because it is "dry" (requiring no chemical development) and therefore compatible with the home or office environment.

The heat required to effect transfer of the colourant is usually supplied by contacting the assembled (but not bonded) donor and receptor sheets with so called "thermal printheads" comprising arrays of miniature electrically-heated elements, each of which is capable of being activated in a timed sequence to provide the desired imagewise pattern of heating. However, such systems provide rather poor resolution and increasing interest is being shown in the use of radiant or projected energy, especially infrared radiation, to supply the heat, thereby taking advantage of the greater commercial availability of laser diodes emitting in the near-infrared region. This is achieved by incorporating a radiation-absorbing material in one of the donor and receptor sheets, normally the former, and subjecting the assembled sheets to an imagewise pattern of radiation. When the assembled sheets are irradiated by radiation of an appropriate wavelength, then the radiation-absorbing material converts the incident energy to thermal energy and transfers the heat to colourant in its immediate vicinity, causing imagewise transfer of the colourant to the receptor.

Examples of thermal transfer media include those disclosed in British Patent No. 1385533; British Patent Publication No. 2083726; European Patent Publication Nos. 403932, 403933, 403934, 404042, 405219, 405296, 407744, 408891, 407907 and 408908; US Patent Nos. 3787210, 3946389, 4541830, 4602263, 4788128, 4904572, 4912083, 4942141, 4948776, 4948777, 4948778, 4950639, 4950640, 4952552 and 4973572; International Patent Publication No. PCT WO 88/04237; Japanese Patent Publication Nos. 21-075292 and 30-043294, and Japanese Patent Nos. 51-088016, 56-082293, 63-319191 and 63-319192.

In the majority of conventional systems using radiant or projected energy to effect the thermal transfer of colourant, the donor sheet comprises a support bearing a donor layer containing the colourant, ordinarily dissolved or dispersed in a binder, with the radiation-absorbing material incorporated in either the same layer as the colourant, e.g., as disclosed in European patent Publication No. 403933, or in a separate underlayer interposed between the support and donor layer, e.g., as disclosed in Japanese Patent No. 63-319191. The donor sheet may be of the diffusion-transfer type (sometimes referred to as "sublimation-transfer" material), whereby colourant is transferred to the receptor in an amount proportional to the intensity of radiation absorbed, or the mass-transfer type, whereby either 0% (zero) or 100% transfer of colourant takes place, depending on whether the absorbed energy reaches a threshold value. In mass-transfer materials, both the colourant and binder are transferred to the receptor sheet.

Two distinct methods are known in which radiation is used to effect thermal transfer of a colourant. In the first method, a laser is scanned directly over the assembled donor and receptor sheets, while its intensity is modulated in accordance with digitally stored image information. This method is disclosed in, e.g.: Research Disclosure No. 142223 (February 1976); Japanese Patent No. 51-88016; U.S. Patent No. 4973572; British Patent No. 1433025, and British Patent Publication No. 2083726.

The second method involves flood exposure from a momentary source, such as a xenon flash lamp, through a suitable mask held in contact with the assembled donor and receptor sheets. This method is disclosed in, e.g: Research Disclosure No. 142223 (February 1976); U.S. Patent Nos. 3828359, 4123309, 4123578 and 4157412, and European Patent Publication No. 365222.

U.S. Patent Nos. 4123309, 4123578 and 4147412 disclose a composite strip material for use in the preparation of art graphics and the like comprising (a) an accepting tape having a layer of a latent adhesive material and (b) a transfer tape having a donor web carrying a lightly adhered layer of microgranules in face-to-face contact with the adhesive layer. At least one of the microgranule and adhesive layers bears a radiation-absorbing pigment. Upon momentary exposure to a pattern of radiation, the pigment is selectively heated, momentarily softening the adjacent portions of the adhesive layer which, upon solidification, adhere to the microgranules. The accepting and transfer tapes are then separated, with the transferring microgranules adhering to the accepting tape only in the irradiated areas.

The pigment is preferably incorporated into the microgranule-containing layer of the transfer tape, thereby providing a direct conductive path to the surface of the adhesive layer. The pigment also serves as a colouring material for the microgranules, with dark coloured microgranules giving dark graphics. Where graphics of a light colour are desired, microgranules of that light color may be used in combination with an accepting tape which comprises a receiving web, a coating of pigment on the receiving web, and a thin layer of adhesive material adhered to the pigment coating. No advantage is taught for placing the pigment in the receptor sheet (other than the visibility of light coloured graphics) and indeed this is said to cause a drop in sensitivity.

A xenon flash lamp which produces broad spectrum bluish-white light in a flash is the preferred exposure source, with the desired imagewise pattern of radiation provided by exposing the composite strip material through a mask bearing image information. However, there are several disadvantages associated with this method of imaging. Xenon flash lamps tend to be bulky, have high power consumption and pose heat dissipation problems, but more importantly, it is very difficult in practice, to obtain large area images of high quality by this method without damaging the mask bearing the image information. This is because, under normal circumstances, the opaque areas of the mask are themselves absorbing and, since the entire area of the mask is illuminated, a large amount of energy is absorbed by the mask with no means by which it can be dissipated quickly. Consequently, high temperatures are generated within the mask, leading to melting or distortion. As the energy absorbed is proportional to the area exposed, the problem becomes more acute with larger-sized images.

In addition, because a xenon lamp is a broad band emitter, the use of a xenon flash exposure generally necessitates the use of carbon black and other materials having a similarly broad absorption as the radiation-absorber, in order to make effective use of the available energy. However, the current trend is to substitute infrared-absorbing dyes for carbon black in pursuit of higher resolution, and also in order to reduce the likelihood of image contamination by the radiation-absorber, e.g., as disclosed in European Patent Publication Nos. 312923, 403930, 403931, 403932, 403933, 403934, 404042, 405219, 405296, 407744, 408891, 408907 and 408908. since dyes have a relatively narrow absorption band, higher intensity xenon flashes are required, which compounds the heat-distortion problem described earlier.

Japanese Patent No. 3-043294 discloses the use of an infrared-absorbing material in a separate sheet which is held in face-to-face contact with a heat-sensitive medium, but there is no disclosure of thermal transfer as described herein.

JP-A-4153087 discloses image receiving materials for use in sublimation thermal transfer or melting thermal transfer in which a light/heat conversion layer and a thermal image receiving layer are positioned on an image receiving support.

Thermal transfer donor sheets comprising a layer of an organic or inorganic colourant vapor-deposited on a controlled-release layer are disclosed, respectively, in U.S. Patent Application Serial Nos.
07/775782 (US-A-5139598) and 07/776602, filed October 11th, 1991. Only thermal printhead imaging is taught in connection with these materials.

U.S. Patent Nos. 4599298 and 4657840 disclose radiation sensitive imaging materials comprising (sequentially): (i) a support, (ii) a vapor-deposited colourant layer, and (iii) a vapor-deposited layer of a metal, metal oxide or metal sulphide. Layer (iii) may be ablated imagewise using a laser, and the exposed areas of layer (ii) may be transferred to a receptor by application of heat, e.g., by direct contact with a heated platen or roller.

European Patent Publication No. 125086 discloses photoresistive elements comprising (sequentially): (i) a support, (ii) a vapor-deposited colourant layer, and (iii) a photoresist overlayer. The imagewise exposed elements are subjected to a development step to remove the resist layer in either the exposed or unexposed regions of the element, depending on whether the resist material is positive or negative-acting, and uniformly heated, e.g., by direct contact with a heated platen, to effect the selective transfer of the colourant. A receptor may receive the transferred colourant or the element with the dye selectively removed can be used as the final image. The colourant can also be transferred without development where the permeability of the resist layer to the colourant is changed on exposure.

The present invention seeks to provide alternative thermal transfer methods and thermal transfer materials.

According to one aspect of the present invention, there is provided a method of thermal transfer imaging which comprises the following steps:
(a) contacting a receptor sheet and a donor sheet having a donor layer comprising a thermally transferable colourant such that the donor layer is in intimate contact with the receptor sheet, one of the donor and receptor sheets comprising a radiation-absorbing material capable of absorbing radiation from an exposure source such that imagewise exposure of the contacted sheets causes heating in the exposed regions, said heating causing thermal transfer of colourant from the donor sheet to the receptor sheet in an imagewise fashion, and
(b) imagewise exposing the contacted donor and receptor sheets using a scanning exposure source, wherein the donor layer of the donor sheet comprises a layer of a vapor-deposited colourant.

The method of the invention utilises a scanning exposure source, such as a laser, to effect the thermal transfer of colourant from a donor sheet to a receptor sheet. "Colourant" is used herein in its broadest sense, as covering any material capable of modifying the surface of the receptor and regardless of whether the modification is visible to the naked eye.

In one aspect of the present invention, the radiation-absorbing material is incorporated in the receptor sheet. The inclusion of the radiation-absorbing material in the receptor sheet offers significant advantages over conventional thermal transfer materials, in which the radiation-absorbing material is present in the donor sheet, both in terms of higher resolution and greater sensitivity, since the heating effect is induced directly in the receptor. In a preferred embodiment, the receptor sheet includes a receptor layer for thermally transferred colourant, with the radiation-absorbing material containing in the receptor layer or, more preferably, in an ordinarily adjacent underlayer thereto.

The donor sheets may be of the diffusion-transfer (sublimation-transfer) type, whereby colourant is transferred to the receptor sheet in an amount proportional to the intensity of the energy absorbed (giving a continuous tone image), but are preferably of the mass-transfer type, whereby essentially 0 (zero) or 100% transfer of colourant takes place depending on whether the absorbed energy exceeds a threshold value.

Mass-transfer donor sheets have several advantages, such as the provision of matched positive and negative images (on the donor and receptor sheet respectively), saturated colours, and the ability to image large areas with a uniform optical density, and are well-suited to half-tone imaging. However, poor resolution and high energy requirements have hampered their use in conventional thermal transfer imaging systems. The method of the invention is capable of producing mass-transfer images of unexpectedly high resolution and low energy requirement.

The mass-transfer materials comprise a support bearing a vapor-deposited colourant layer, preferably separated by a controlled release layer, as disclosed in U.S. Patent Applications Serial Nos. 07/775782 (US-A-5139598) and 07/776602, filed October 11th, 1991. These donor sheets are found to give high resolution images with good colour saturation, high transparency and uniform optical density.

According to another aspect of the invention there is provided a thermal transfer medium comprising a donor sheet having a donor layer comprising a vapor-deposited thermally transferable colourant and a receptor sheet comprising a radiation-absorbing material. The donor support may optionally have a controlled release layer (described hereinafter) onto which the colourant is vapor-deposited.

The radiation-absorbing material may be contained in a separate, dedicated layer (referred to herein as a "radiation-absorbing layer"), e.g., in an underlayer to the vapor-deposited colourant layer in the donor sheet or any receptor layer(s) in the receptor sheet. Alternatively, the radiation-absorbing material may be included in one of the other component layers of the donor or receptor sheets, e.g., the receptor layer of the receptor sheet. Where the colourant is itself radiation-absorbing such that it is to be regarded as the radiation-absorbing material, then no other radiation-absorbing material is required.

The radiation-absorbing material, ordinarily absorbing radiation in the wavelength region 600 to 1070 nm, more usually 750 to 980 nm, may comprise any suitable material able to absorb the radiant energy of the exposing source, convert it to heat energy and transfer that energy to the colourant in its immediate vicinity. Examples of suitable radiation-absorbing materials include pigments, such as carbon black, e.g., as disclosed in British Patent No. 2083726, and dyes, including: (but not limited to): phthalocyanine dyes, e.g., as disclosed in U.S. Patent No. 4942141; ferrous complexes, e.g., as disclosed in U.S. Patent No. 4912083; squarylium dyes, e.g., as disclosed in U.S. Patent No. 4942141; chalcogenopyrylo-arylidene dyes, e.g., as disclosed in U.S. Patent No. 4948776; bis(chalcogenopyrylo)polymethine dyes, e.g., as disclosed in U.S. Patent No. 4948777; oxyindolizine dyes, e.g., as disclosed in U.S. Patent No. 4948778; bis(aminoaryl)polymethine dyes, e.g., as disclosed in U.S. Patent No. 4950639; merocyanine dyes, e.g., as disclosed in U.S. Patent No. 4950640; tetraarylpolymethine dyes; dyes derived from anthraquinones and naphthaquinones, e.g., as disclosed in U.S. Patent No. 4952552; cyanine dyes, e.g., as disclosed in U.S. Patent No. 4973572; trinuclear cyanine dyes, e.g., as disclosed in European Patent Publication No. 403933; oxonol dyes, e.g., as disclosed in European Patent Publication No. 403934; indene-bridged polymethine dyes, e.g., as disclosed in European Patent Publication No. 407744, and nickel-dithiolene dye complexes, e.g., as disclosed in European Patent Publication No. 408908, and croconium dyes, e.g., as disclosed in EP-A-568267.

The radiation-absorbing material is preferably present in an amount and distribution sufficient so that absorption of the exposing radiation by the material will locally generate sufficient heat to enable transfer of the colourant from the donor sheet to the receptor sheet. The amount of radiation-absorbing material required for efficient colourant transfer will vary widely depending on the nature of the material used etc., but it is preferably present in an amount sufficient to provide a transmission optical density of at least 1.0 absorbance units, more preferably at least 1.5 absorbance units at the wavelength of the exposing radiation.

The radiation-absorbing layer ordinarily comprises a binder layer having dissolved or dispersed therein the radiation-absorbing material. Where applicable, the binder of the radiation-absorbing layer may comprise any of a number of suitable materials including: poly(vinyl acetals), such as poly(vinyl formal) and poly(vinyl butyral); polycarbonates; poly(styrene-acrylonitrile); polysulfones; poly(phenylene oxide); poly(vinylidene chloride-vinyl acetate) copolymers, and mixtures thereof, although binder materials having a glass-transition temperature (T_{g}) of greater than 100°C are preferred to ensure that the colourant adheres to the receptor sheet/layer and not the radiation-absorbing layer during thermal transfer.

When the radiation-absorbing layer comprises a mixture of dye or pigment and a binder, it is normally coated as a solution or dispersion in a suitable solvent, e.g., lower alcohols, ketones, esters, chlorinated hydrocarbons, and mixtures thereof. Any of the well-known solvent-coating techniques may be used, such as knife-coating, roller-coating, wire-wound bars etc. The thickness of the radiation-absorbing layer must be sufficient to provide the necessary optical density, and will depend on factors such as the extinction coefficient of the dye or pigment used, and its solubility in the binder. Relatively thin layers (e.g., up to 5µm dry thickness) are preferred.

Alternatively, the radiation-absorbing layer may comprise a continuous layer of a solid, radiation-absorbing pigment or dye without a binder. A particularly suitable pigment in this context is "black aluminium oxide", which is a graded mixture of aluminium and aluminium oxide. Layers of this materials may be formed by vapour depositing aluminium metal in the presence of controlled amounts of oxygen, as disclosed in U.S. Patent Nos. 4430366 and 4364995. Very thin (<1µm) coatings of this material show a high optical density over a wide wavelength range, covering the visible and infrared, which ensures compatibility with a wide range of exposure sources.

Receptor sheets for thermally transferred colourant normally comprises a support sheet having coated on at least one major surface thereof a receptor layer, ordinarily comprising a heat-softenable (low T_{g}), usually thermoplastic, binder, but when the radiation-absorbing material is present in the receptor layer, then the binder may require a higher T_{g}, typically 100°C or greater. Ideally, the binder should soften during the imaging process to an extent that is sufficient to induce transfer of the colourant, but is not so great as to cause ablation, lateral flow or transfer to the donor sheet. This is more likely to be a problem when the radiation-absorbing material is present in the receptor layer. In these circumstances, the choice of binder is governed to a large extent by the nature of the donor sheet being used. For example, where the donor sheet comprises a layer of vapor-deposited dye or pigment, it is found that low T_{g} receptor layers (containing the radiation-absorbing material) are unsuitable for the reasons outlined above, whereas high T_{g} layers give good results.

When the radiation-absorbing material is present in a separate underlayer, that is, a layer interposed between the support and, ordinarily adjacent, the receptor layer, it is preferably coated in a high T_{g} binder, typically having a T_{g} of greater than 90°C, with the receptor (over)layer comprising a lower T_{g} material having, e.g., a T_{g} of from 40 to 90°C. Preferred high T_{g} binders include polyesters and polycarbonates, e.g., bisphenol-A polycarbonate.

The receptor layer may comprise, e.g., a polycarbonate, a polyurethane, a polyester, a poly(vinyl chloride), poly(styrene-acrylonitrile), poly(ethylene-acrylic acid), poly(caprolactone), poly(vinylidene chloride-vinyl acetate) or a mixtures thereof. The receptor layer may be present in any amount which is effective for the intended purpose.

Where the desired image is that transferred to the receptor sheet, then if the radiation-absorbing material is present in the receptor sheet, it is preferably colourless to the human eye or is photobleachable, so as to avoid "staining" the image. Where the final image is that remaining on the donor, or when the image on the receptor is subsequently transferred to a second receptor, such considerations are unimportant. Examples of radiation-absorbers with reduced staining properties include phthalocyanines (e.g., as disclosed in U.S. Patent No. 4788128): nickel-dithiolene complexes (e.g., as disclosed in European Patent Publication No. 408908), and croconium dyes (e.g., as disclosed in EP-A-568267).

Where the desired image is that transferred to the receptor sheet, then the receptor layer may, subsequent to imaging, be separable from the layer containing the radiation-absorbing material.

The support of the receptor can be made of any material to which an image receptive layer can be adhered, includes materials that are smooth or rough, transparent or opaque, flexible or rigid and continuous or sheetlike. The material should be able to withstand the heat required to transfer the colourant without decomposing or distortion. Of course at least one of the donor and receptor sheets must be transparent to the exposing radiation to allow for irradiation of the radiation-absorbing material, with the support material chosen accordingly. Suitable support materials are well known in the art, representative examples of which include (but are not limited to): polyesters, especially poly(ethylene terephthalate) and poly(ethylene naphthalate); polysulfones; polyolefins, such as poly(ethylene), poly(propylene) and poly(styrene); polycarbonates; polyimides; polyamides; cellulose esters, such as cellulose acetate and cellulose butyrate; poly(vinyl chloride), and derivatives thereof. A preferred support material is white-filled or transparent poly(ethylene terephthalate) or opaque paper. The support may also be reflective, such as baryta-coated paper, ivory paper, condenser paper, or synthetic paper. The support generally has a thickness of 0.05 to 5mm, with 0.05mm to 1mm preferred.

The receptor (and where appropriate the donor) support may contain fillers, such as carbon black, titania, zinc oxide and dyes, and may be treated or coated with those materials generally used in the formation of films, such as coating aids, lubricants, antioxidants, ultraviolet radiation absorbers, surfactants, and catalysts.

In accordance with the present invention the donor sheet comprises a layer of a vapor-deposited colourant and either the colourant itself constitutes the radiation-absorbing material such that it will transfer unaided on irradiation of the assembled donor and receptor sheets, or the donor sheet further comprises a radiation-absorbing material in a separate, ordinarily adjacent, underlayer to the colourant layer, or the receptor comprises a radiation-absorbing material.

The use of a vapor-deposited colourant donor layer offers significant advantages over conventional thermal transfer donor materials, in which the colourant is dissolved or dispersed in a binder, both in terms of higher resolution and greater sensitivity (speed). A vapor-deposited colourant is free from contamination by binder materials and produces a pure, more intense image on the receptor sheet. Also the transferred image shows a highly uniform optical density, even when large areas are transferred.

Colourants from any chemical class that may be vapor-deposited, i.e., which do not decompose upon heating, may be used. Preferred organic colourants include (but are not limited to): copper phthalocyanine and Pigment Yellow PY17 (commercially available from Sun Chemical Corporation) and Pigment violet PV19 (commercially available from Ciba Geigy Corporation). Preferred inorganic colourants include (but are not limited to): metals, such as aluminium, copper, gold, silver etc., and metal oxides, especially "black aluminium oxide", as disclosed in U.S. Patent Nos. 4430366 and 4364995, which gives a neutral black colour.

The vapor-deposited colourant layer is preferably coated at a sufficient thickness to provide a transmission optical density of at least 0.5 absorbance units, preferably at least 1.0 absorbance units. The thickness of the colourant layer depends upon the colourant used and the desired minimum optical density, but it can be as thin as a few tens of nanometers or as thick as several micrometers, e.g., 10 to 1000nm thick, preferably 50 to 500nm thick, and more preferably 100 to 400nm thick. The colourant is typically pre-purified by sublimation prior to vapor-deposition.

Techniques for the vapour deposition of colourant layers are well known in the art, and include resistive heating methods, radio frequency sputtering, plasma deposition, chemical vapour-deposition, epitaxy deposition and electron beam deposition methods. Specific examples may be found, e.g., in U.S. Patent Nos. 4430366, 4364995, 4587198, 4599298 and 4657840, and U.S. Patent Application Serial Nos. 07/775782 and 07/776602.

The colourant layer may be continuous or discontinuous, e.g., it may be deposited in the form of a pattern or in the form of alphanumeric characters by use of suitable masking techniques during the vapour deposition. Preferably, the colourant layer is continuous.

In many cases, it is found that the vapour-deposited colourant layer exhibits anisotropic cohesive forces. For example, it may possess a columnar microstructure (as disclosed in US-A-5139598) in which the cohesive forces operating between the columns are substantially smaller than the cohesive forces acting within individual columns. Factors which are believed to affect the microstructure of the deposited layer include the substrate temperature, the deposition rate (which is a function of the evaporation source temperature, the source-to-substrate distance and the substrate temperature), the deposition angles, and the chamber pressure. (See, e.g: Debe and Poirier, "Effect of gravity on Copper Phthalocyanine Thin Films III: Microstructure Comparisons of Copper Phthalocyanine Thin Films Grown in Microgravity and Unit Gravity", Thin solid Films, 186, pp.327 to 347 (1990); and Zurong et al., Kexue Tongbao, Vol. 29, p.280 (1984)). While an anisotropic microstructure is not essential in the practice of the present invention, it is highly preferred, as it is believed to contribute significantly to the resolution of the transferred image.

In the embodiment wherein the colourant layer itself is suitably radiation-absorbing, and a separate radiation-absorbing material is not required, the colourant layer is preferably vapour-deposited onto a controlled release layer present on the support of the donor sheet. Such a layer provides a controlled adhesion between the colourant and the support, such that the colourant transfers readily to the receptor sheet when required, but remains suitably abrasion resistant during normal handling.

Controlled release layers are particularly useful in the case of inorganic colourants, such as black aluminium oxide, which otherwise adhere too strongly to the most commonly used donor supports, and hence require inconveniently high irradiation intensities to effect transfer. Controlled release layers are described in detail in U.S. Patent Application Serial Nos. 07/775782 (US-A-5139598) and 07/776602, and may comprise, e.g., mixtures of two or more polymers that differ markedly in their affinity towards the donor support, or may comprise inorganic particles, such as boehmite (aluminium monohydrate) particles, hydrophobic silica particles, alumina particles, titania particles etc. The latter type of controlled release layer is preferred for use with inorganic colourants, and a particularly preferred controlled release layer for use with black aluminium oxide comprises a coating of boehmite particles, which are available as an aqueous dispersion under the trade name "CATAPAL D" from Vista Chemical Co., Houston, Texas, U.S.A. The former type of controlled release layer is preferred for use with organic colourants.

The support of the donor sheet ordinarily comprises a transparent substrate to allow for irradiation of the radiation-absorbing material by the exposure source. Examples of suitable support materials include (but are not limited): polyether sulfones; polyimides, such as polyimide-amides and polyether imides; polycarbonates; polyacrylates; polysulfones; cellulose ester, such as ethyl cellulose, cellulose acetate, cellulose acetate hydrogen phthalate, cellulose acetate butyrate, cellulose acetate propionate, cellulose triacetate etc.; a poly (vinyl alcohol-vinyl acetal) copolymers; polyester, such as poly(ethylene terephthalate) which may be biaxially stabilized and poly(ethylene naphthalate); fluorinated polymers, such as poly(vinylidene fluoride) and poly(tetrafluoroethylene-hexafluoropropylene); polyvinyl resins, such as poly(vinyl acetate, poly(vinyl chloride); polyethers, such as poly(oxyethylene); polyacetals; such as poly(vinyl butyral) and poly(vinyl formal); polyolefins, such as poly(ethylene), poly(propylene) and poly(styrene), and polyamides. However, where the assembled donor and receptor sheets are exposed through the receptor sheet, then the support material of the receptor may be opaque, contain fillers etc., considerations of transparency being unimportant. The donor support may be flexible or rigid, although the former is preferred, and continuous or sheet-like.

According to a further aspect of the present invention, there is provided a thermal transfer donor sheet comprising (sequentially): a support; a radiation-absorbing layer comprising a dye or the combination of a pigment and a binder, and a layer of a vapor-deposited thermally transferable colourant.

In use, the thermal transfer donor sheet is combined with a receptor sheet and irradiated by radiation of an appropriate wavelength for the radiation-absorbing layer. In the exposed regions of the assembled donor and receptor sheets, the radiation-absorbing layer converts the radiant energy of the exposure source to thermal energy and transfers the heat to the colourant causing the transfer of colourant to the receptor sheet in an imagewise fashion.

The receptor sheet usually comprises a support having coated on at least one major surface thereof a receptor layer, ordinarily comprising a heat-softenable (i.e., T_{g} <100°C), usually thermoplastic, binder - although any suitable receptor for thermally transferred colourant may be used.

Any suitable scanning exposure source may be used to effect the thermal transfer of the colourant from the donor sheet to the receptor sheet, although the preferred exposure source is a laser, with the exposure source and radiation-absorbing material selected such that the output radiation closely matches the wavelength of maximum absorption of the radiation-absorbing material, in order to make effective use of the available energy.

Several different kinds of laser may be used to effect thermal transfer of colourant, including (but not limited to): gas ion lasers, such as argon and krypton lasers; metal vapor lasers, such as copper, gold and cadmium lasers; solid state lasers, such as ruby or YAG lasers, and diode lasers, such as gallium arsenide lasers, but in practice, laser diodes which offer substantial advantages in terms of their small size, low cost, stability, reliability, ruggedness and ease of modulation in accordance with digitally stored information, are preferred. Generally, exposure sources emitting in the infrared region from 750 to 950nm are preferred, although any source emitting radiation in the region 600 to 1070nm may be usefully employed in the practice of the invention.

In one method, the laser is scanned directly over the assembled donor and receptor sheets, while its intensity is modulated in accordance with digitally stored image information. This method is disclosed in, for example: Japanese Patent No. 51-088016, U.S. Patent No. 4973572, British Patent Nos. 1433025, and British Patent Publication No. 2083726, and provides a very good resolution.

Another method of imaging is disclosed in EP 0583165 entitled "Thermal Transfer Imaging" which comprises:
(a) assembling the donor and receptor sheets so that the donor layer of the donor sheet is in intimate contact with the receptor sheet;
(b) contacting a photographic mask with the assembled donor-receptor sheets, and
(c) exposing the assembled donor and receptor through the photographic mask using a scanning, preferably continuous, exposure source so that in areas defined by the transparent regions of the mask, the exposing radiation is absorbed and converted to thermal energy by the radiation-absorbing material to effect the thermal transfer of colourant from the donor sheet to the receptor sheet.

By suitable adjustment of the various parameters, such as laser power, spot size, scan rate and focus position, it is possible to effect thermal transfer imaging without damaging the photographic mask. This is due to the fact that only a small area of the mask is irradiated at any one instant, with the remainder available to act as a heat sink. The optimum exposure parameters depend on a number of variables, such as the sensitivity of the thermal transfer media and the thermal conductivity of both the mask and the radiation absorber. The mask preferably has a thermal conductivity of at least 2x10⁻³Wcm^{-1°}K⁻¹. The assembled donor and receptor sheets preferably constitute a system of sufficient sensitivity to allow the thermal transfer of colourant at energy levels of less than 4J/cm².

Where the colourant layer is present in the donor sheet as a discontinuous layer, e.g., as a pattern or as alphanumeric characters, simple illumination with a continuous, scanning laser is sufficient without the need of a mask.

Whichever method of address is used, the laser preferably has a power of at least 5mW, with the upper power limit depending on the characteristics of the mask (if used) and the thermal transfer media, as well as the scan speed and spot size. The laser is focused on the radiation-absorbing layer to give an illuminated spot of small, but finite dimensions, which is scanned over the entire area to be imaged. Exposure of the assembled donor and receptor sheets may be carried out from either side, i.e., through the support of the donor sheet, or through the support of the receptor sheet, providing of course that all layers through which the radiation must pass before reaching the radiation-absorbing material are suitably transparent. In the case of exposure through a mask, the laser output may be adjusted via a cylindrical lens to a narrow line, the longer dimension of which is perpendicular to the direction of scan, thereby permitting a larger area to be scanned in one pass. Scanning of the laser may be carried out by any of the known methods, but will normally involve raster scanning, with successive scans abutting or overlapping as desired. Two or more lasers may scan different areas of a large image simultaneously.

To ensure good resolution and effective image transfer, it is essential that the donor and receptor sheets and the mask (if used) are held in intimate contact with each other during imaging. This is achieved by subjecting the assembly of mask (if used) and donor and receptor sheets to pressure, ordinarily of at least 10g/mm², preferably at least 40g/mm² and typically about 100g/mm².

Multicolour images may be produced by repeating the above described imaging methods with successive donor sheets of different colours, using the same receptor in each case.

If desired, the final image may be transferred from the original receptor to another substrate, such as paper or card stock. This transfer may be carried out by conventional thermal lamination techniques, as disclosed in, e.g., European Patent Publication No. 454083. If the receptor support is transparent, then radiation-induced transfer is also possible.

The present invention will now be described with reference to the accompanying, non-limiting Examples in which the following resins are used as binder materials for the various layers of the donor/receptor sheets. BIS A is bisphenol-A-polycarbonate of the formula: having a glass-transition temperature (Tg) of 160°C - commercially available from Polysciences Inc.

CAB 381-20 is cellulose acetate butyrate having a Tg of 138°C - commercially available from Eastman Kodak.

CAB 500 is cellulose acetate butyrate having a Tg of 96°C - commercially available from Eastman Kodak.

VINYLITE VYNS is a poly(vinylidene chloride-vinyl acetate) copolymer having a Tg of 79°C - commercially available from Union Carbide.

BUTVAR B-76 is a poly(vinyl butyral) resin having a Tg of 56°C - commercially available from Monsanto.

### Example 1

This Example demonstrates how a scanning exposure source, such as a laser, can be used to effect thermal transfer of colourant from a donor sheet to a receptor sheet comprising a support bearing a receptor layer for thermally transferred colourant, the receptor sheet further comprising a radiation-absorbing material in either the receptor layer (Receptor Sheets 1 to 3) or in a separate underlayer interposed between the support and receptor layer (Receptor Sheets 4 to 7).

Receptor sheets 1 to 7 were prepared as follows:-

### Receptor Sheet 1

Support: poly(ethylene terephthalate) polyester (100 µm thick)

Receptor Layer: a solution of VINYLITE VYNS (1.5g) and IR-Dye I(0.05g) dissolved in a mixture (10g) of methylethylketone and toluene (1:1) was coated onto the support at a wet thickness of 37.5µm.

### Receptor Sheet 2

Support: as per Receptor Sheet 1.

Receptor layer: a solution of CAB 500 (1g) and IR-Dye I (0.05g) dissolved in a mixture (10g) of methylethylketone and toluene (1:1).

### Receptor Sheet 3

Support: as per Receptor Sheet 1.

Receptor layer: a solution of BIS A (3g) and IR-Dye I (0.1g) dissolved in a mixture (30g) of cyclohexanone and dichloromethane (3:2).

### Receptor Sheet 4

Support: as per Receptor Sheet 1.

IR-absorbing layer: a mixture of BIS A (6.7g) and IR-Dye 1 (0.05g) in dichloromethane (53.2g) and cyclohexanone (6.7g) was coated onto the support at a wet thickness of 25 µm.

Receptor layer: a solution of BUTVAR B-76 (1g) in a mixture (10g) of methyl ethyl ketone and methanol (1:1) was coated at Kbar 1 onto the dried IR-absorbing layer. "Kbars" are wire wound coating rods, commercially available from R.K. Print Coat Instruments Ltd.

### Receptor Sheet 5

Support: as per Receptor Sheet 1.

IR-absorbing layer: as per Receptor Element 4.

Receptor layer: a solution of VINYLITE VYNS (1.5g) dissolved in a mixture (10g) of methylethylketone and toluene (1:1) was coated at Kbar 1 onto the dried IR-absorbing layer.

### Receptor Sheet 6

Support: as per Receptor Sheet 1.

IR-absorbing layer: as per Receptor Element 4.

Receptor layer: a solution of CAB 500(1g) dissolved in a mixture (10g) of methylethylketone and methanol (1:1) was coated at Kbar 1 onto the dried IR-absorbing layer.

### Receptor Sheet 7

Support: as per Receptor Sheet 1

IR-absorbing layer: as per Receptor Element 4.

Receptor layer: a solution of CAB 381-20 (1g) dissolved in a mixture (10g) of methylethylketone and methanol (1:1) was coated at Kbar 1 onto the dried IR-absorbing layer.

A sample of each of Receptor Sheets 1 to 7 was placed in face-to-face contact with the following donor sheet, with the donor layer of the donor sheet in intimate contact with the receptor layer of the receptor sheet.

### Donor Sheet A

Support: poly(ethylene terephthalate) polyester base (100 µm thick).

Donor layer: a copper phthalocyanine pigment commercially available from Sun chemicals Inc., was purified by vacuum sublimation at 500°C and 200Nm⁻² (1.5 Torr) (argon) pressure. The purified pigment was loaded in a heater made from stainless steel sheet material and the heater positioned in a custom built 30cm bell jar vacuum coater equipped with a diffusion pump and a 15cm web drive, about 4cm below the web. The support was fed onto the web drive before pumping the vacuum chamber down to 6.7x10⁻³Nm⁻² (5x10⁻⁵Torr) pressure. The heater was heated to 410°C using an applied a.c. power supply to vaporise and deposit the pigment onto the support, the web drive moving at a speed of 0.25cm per second.

Each of the contacted donor and receptor sheets was overlaid with a UGRA line dot scale mask and addressed with a laser diode emitting at 830 nm using the imaging assembly described hereinafter with reference to Figure 1.

The assembled donor and receptor sheets (with mask) are sandwiched between a transparent pressure plate (2) and a support roller (4) biased against the plate (2) by a suitable weight (6) acting through pivot (8). A mirror (10) and focusing lens (12) mounted on a support (14) are provided to focus the beam (16) from the laser diode (18) onto the IR-absorbing layer of the receptor sheet at the point of maximum pressure provided by the support roller (4). A linear stepped motor drive (20) advances the support (14) along slides (22). The assembly of donor and receptor sheets was imaged at a power level sufficient to produce maximum effect on the donor sheet, but with minimum IR-induced heating in the UGRA half-tone mask. The operating conditions were as follows: laser power 10mW, spot size 20µm, scan rate 1.5cm per second and a contact pressure (between support roller (4) and pressure plate (2)) in excess of 50gmm⁻². This method of contact exposing imaging materials via half-tone masks with monochromatic radiation is disclosed in EP 0583165. After exposure, each composite was separated and the percentage (%) dot transfer and the resolved dot range estimated at a resolution of 60 lines per cm. The results are shown in TABLE 1 below.

**TABLE 1**

| Assembly | Receptor Sheet | Donor Sheet | Dot Transfer (%) | Resolved Dot Range |
|---|---|---|---|---|
| 1 | 1 | A | 0 | - |
| 2 | 2 | | 0 | - |
| 3 | 3 | | 100 | 97/3 |
| 4 | 4 | | 100 | 97/3 |
| 5 | 5 | | 100 | 97/3 |
| 6 | 6 | | 0 | - |
| 7 | 7 | | 0 | - |

Assemblies 1 to 3: demonstrate that, where the donor sheet comprises a vapor-deposited colourant layer and the radiation-absorbing material is present in the receptor layer of the receptor sheet, then the binder for the latter should desirably have a high glass-transition temperature (Tg) typically greater than 100°C. The use of lower Tg materials, such as VINYLITE VYNS and CAB 500, results in much binder flow and possible ablation, such that mass transfer from the donor sheet is prevented.

Assemblies 4 to 7: demonstrate that the provision of the radiation-absorbing material in an underlayer to the receptor layer permits mass transfer from the donor sheet to the receptor sheet in a clean (100% transfer) manner. The best results were obtained from binders having a Tg of from 40 to 90°C, as materials, such as CAB 381-20 and CAB 500, having a Tg greater than 90°C do not melt/soften sufficiently to allow mass transfer.

### EXAMPLE 2

This Example demonstrates how a scanning exposure source can be used to effect thermal transfer from a donor sheet comprising a layer of a vapor-deposited colourant wherein either the colourant is capable of absorbing the exposing radiation (Donor Sheet D) or a separate radiation-absorbing material is present in an underlayer adjacent the colourant layer (Donor Sheets B, C and E).

Donor Sheets B to E where as follows:

### Donor Sheet B

Support: poly(ethylene terephthalate) polyester base (100µm thick).

IR-absorbing layer: IR-Dye I (0.05g) was added to BIS-A (3.3g) in dichloromethane (26g) and cyclohexanone (3.3g) and the resulting mixture tumble-stirred for 24 hours. The mixture was coated at 37.5µm wet thickness onto the support and dried at room temperature. Care was taken to ensure that dust particles did not deposit on the coating. The transmission optical density of the IR-absorbing layer was measured as 1.2 absorbance units at 830nm.

Colourant layer: as per donor layer of Donor Sheet A of Example 1.

### Donor Sheet C

Support: as per Donor Sheet B.

IR-absorbing layer: as per Donor Sheet B.

Colourant layer: violet pigment PV19 - commercially available from Ciba Geigy, was purified by vacuum sublimation at 475°C and 2.7Nm⁻² (20 mTorr) pressure as detailed above. The purified pigment was vapor-deposited onto the coated support under virtually identical deposition conditions but using a heater temperature of 400°C.

### Donor Sheet D

Support: poly(ethylene terephthalate) polyester base (75µm thick).

IR-absorbing/Colourant layer: a boehmite (Al0.0H) subbing layer (0.4% by weight CATAPAL D, commercially available from Vista Chemical Co.; 10µm wet thickness) was coated onto the support, dried at 80°C and overcoated with a vapor-deposited layer of "black aluminium oxide" (approximately 0.15µm thick), following the procedure described in U.S. Patent Nos. 4364995 and 4430366. The transmission optical density of the layer was determined to be at least 4.6 absorbance units.

### Donor Sheet E

Support: as per Donor Sheet D.

IR-absorbing layer: as per Donor Sheet D.

Colourant layer: as per Donor Sheet B.

A sample of each of Donor Sheets B to E was placed in face-to-face contact with Receptor Sheets 8 and 9 (see below), with the donor layer of the donor sheet in intimate contact with the receptor layer of the receptor sheet.

### Receptor Sheet 8

Support: paper base.

Receptor layer: a layer (1.5µm thick) of a poly(ethylene-acrylic acid) emulsion (Tg=34°C), commercially available from Schering was coated on to the support.

### Receptor Sheet 9

Support: poly(ethylene terephthalate) polyester (100 µm thick).

Receptor layer: a layer (1.5µm thick) of a poly(vinylidene chloride-vinyl acetate) resin (Tg=79°C), commercially available from Union Carbide under the trade name VINYLITE VYNS, was coated onto the support.

Each of the contacted donor and receptor sheets was overlaid with a UGRA line dot scale mask and imaged as described in Example 1, but using the following operating conditions: laser energy 10mW, spot size 10µm, scan rate 1.5cm per second and a contact pressure (between support roller and pressure plate) of 50gmm⁻². After exposure, the donor and receptor sheets were separated and the percentage (%) dot transfer and the resolved dot range estimated at a resolution of 60 lines per cm. The results are shown in TABLE 2.

**TABLE 2**

| Donor Sheet | Receptor Sheet | | | |
|---|---|---|---|---|
| | 8 | | 9 | |
| | Dot Transfer (%) | Resolved Dot Range | Dot Transfer (%) | Resolved Dot Range |
| B | 100 | 95/5 | 100 | 97/3 |
| C | 100 | 95/5 | 100 | 97/3 |
| D | 100 | 97/3 | patchy* | - |
| E | 100 | - | 100 | - |

| | | | | |
|---|---|---|---|---|
| * The receptor layer (VINYLITE VYNS) tended to lose adhesion to the support and adhere to the black aluminium oxide donor layer of the donor sheet. | | | | |

The degree of dot transfer was, in the majority of cases, excellent (100% transfer) with good resolution, yielding matched positive and negative images on the donor and receptor sheet, respectively. The images were also characterised by a high uniformity of optical density over large areas.

### GLOSSARY

"VINYLITE VYNS" (Union Carbide), "CATAPAL D" (Vista Chemical Co.), "PV17" and "PV19" (Ciba Geigy), "BUTVAR" (Monsanto), "CAB" (Eastman Kodak), "BIS A" (Polysciences), are all trade names/designations.

## Claims

1. A methods of thermal transfer imaging which comprises the following steps:
(a) contacting a receptor sheet with a donor sheet having a donor layer comprising a thermally transferable colourant such that the donor layer is in intimate contact with the receptor sheet, one of the donor and receptor sheets comprising a radiation-absorbing material capable of absorbing radiation from an exposure source such that imagewise exposure of the contacted sheets causes heating in the exposed regions, said heating causing thermal transfer of colourant from the donor sheet to the receptor sheet in an imagewise fashion, and
(b) imagewise exposing the contacted sheets using a scanning exposure source,
CHARACTERISED IN THAT
the donor layer comprises a layer of a vapor-deposited colourant.

2. A method as claimed in Claim 1 in which the receptor comprises a support having coated thereon a receptor layer for the colourant and the radiation-absorbing material is present in either the receptor layer or a separate underlayer thereto.

3. A method as claimed in Claim 2 in which the receptor layer comprises a layer of a binder having dissolved or dispersed therein the radiation-absorbing material.

4. A method as claimed in Claim 2 in which the receptor sheet comprises a support having sequentially coated thereon a radiation-absorbing layer comprising the radiation-absorbing material and as an overlayer thereto the receptor layer.

5. A method as claimed in Claim 1 in which the vapor-deposited thermally transferable colourant is capable of absorbing the exposing radiation such that it will transfer unaided on exposure of the contacted sheet.

6. A method as claimed in any preceding Claim in which the donor sheet comprises a support bearing a controlled release layer onto which the colourant is vapor-deposited.

7. A method as claimed in Claim 1 in which the donor sheet comprises a support having sequentially coated thereon a radiation-absorbing layer comprising the radiation-absorbing material followed by a layer of vapor-deposited thermally transferable colourant.

8. A method as claimed in any preceding Claim in which the colourant layer is vapor-deposited as a film of anisotropic topography.

9. A method as claimed in any one of Claims 1 to 4, 6 and 7 in which the radiation-absorbing material is selected from carbon black and other pigments; nickel-dithiolene dye complexes; ferrous complexes; cyanine dyes; merocyanine dyes; oxyindolizine dyes; indene-bridged polymethine dyes; trinuclear cyanine dyes; bis(aminoaryl)polymethine dyes); tetraarylpolymethine dyes; chalcogenopyrylo-arylidene dyes; bis(chalcogenopyrylo)polymethine dyes; phthalocyanine dyes; squarylium dyes; dyes derived from anthraquinones and naphthaquinones, and croconium dyes.

10. A method as claimed in any preceding Claim in which the thermally transferable colourant is a dye or pigment.

11. A method as claimed in Claim 10 in which the colourant is an organic colourant or an inorganic pigment selected from metals, metal oxides and mixtures thereof.

12. A method as claimed in any preceding Claim in which step (b) further comprises: assembling a photographic mask in intimate contact with the contacted donor and receptor sheets and exposing the assembly through the photographic mask, the exposing radiation effecting thermal transfer of colourant from the donor sheet to the receptor sheet in areas defined by the transparent regions of the mask.

13. A method as claimed in Claim 12 in which a pressure of at least 10g/mm² is applied to the assembly of photographic mask and donor and receptor sheets.

14. A method as claimed in Claim 12 or Claim 13 in which the contacted donor and receptor sheets constitute a system which is sufficiently sensitive to effect transfer of colourant at energy levels of less than 4J/cm².

15. A method as claimed in any preceding Claim in which the scanning exposure source is a laser or laser diode.

16. A method as claimed in Claim 15 in which the laser has a power of at least 5mW.

17. A thermal transfer donor sheet comprising sequentially: a support; a radiation-absorbing layer comprising a dye or the combination of a pigment and a binder, and a layer of a vapor-deposited thermally transferable colourant.

18. A thermal transfer donor sheet as claimed in Claim 17 in which the radiation-absorbing material absorbs radiation having a wavelength of from 600 to 1070nm.

19. A thermal transfer donor sheet as claimed in Claim 17 or Claim 18 in which the radiation-absorbing layer comprises a layer of a binder having dissolved or dispersed therein the radiation-absorbing material.

20. A thermal transfer donor sheet as claimed in Claim 19 in which the binder of the radiation-absorbing layer has a glass-transition temperature (T_{g}) of at least 100°C.

21. The combination of a thermal transfer donor sheet as claimed in any one of Claims 17 to 20 and a receptor for said thermally transferable colourant.

22. A thermal transfer medium comprising a donor sheet having a donor layer comprising a layer of a vapor-deposited thermally transferable colourant and a receptor sheet for thermally transferred colourant comprising a radiation-absorbing material.

## Patentansprüche

1. Verfahren zur thermischen Bildübertragung, umfassend die folgenden Schritte:
(a) Inkontaktbringen eines Rezeptorblattes mit einem Donorblatt, umfassend eine Donorschicht, die ein thermisch übertragbares Färbemittel umfaßt, so daß sich die Donorschicht in engem Kontakt mit dem Rezeptorblatt befindet, wobei eines der Donor- und Rezeptorblätter ein Strahlung absorbierendes Material umfaßt, das Strahlung einer Belichtungsquelle absorbieren kann, so daß eine bildweise Belichtung der in Kontakt befindlichen Blätter eine Erwärmung in den belichteten Bereichen bewirkt, wobei die Erwärmung eine bildweise thermische Übertragung von Färbemittel vom Donorblatt zum Rezeptorblatt bewirkt, und
(b) bildweise Belichtung der in Kontakt befindlichen Blätter unter Verwendung einer Scanning-Belichtungsquelle,
dadurch gekennzeichnet, daß
die Donorschicht eine Schicht eines aus der Gasphase abgeschiedenen Färbemittels umfaßt.

2. Verfahren nach Anspruch 1, wobei der Rezeptor einen Träger umfaßt, auf dem eine Rezeptorschicht für das Färbemittel aufgebracht ist, und wobei das Strahlung absorbierende Material entweder in der Rezeptorschicht oder in einer getrennten Unterschicht dazu vorhanden ist.

3. Verfahren nach Anspruch 2, wobei die Rezeptorschicht eine Schicht eines Bindemittels umfaßt, in dem das Strahlung absorbierende Material gelöst oder dispergiert ist.

4. Verfahren nach Anspruch 2, wobei das Rezeptorblatt einen Träger umfaßt, auf dem nacheinander eine, das Strahlung absorbierende Material umfassende, Strahlung absorbierende Schicht und die Rezeptorschicht als Deckschicht darauf aufgebracht sind.

5. Verfahren nach Anspruch 1, wobei das aus der Gasphase abgeschiedene, thermisch übertragbare Färbemittel die Belichtungsstrahlung absorbieren kann, so daß es bei der Belichtung des in Kontakt befindlichen Blattes ohne Hilfsmittel übertragen wird.

6. Verfahren nach einem der vorstehenden Ansprüche, wobei das Donorblatt einen Träger mit einer Schicht zur regulierten Freisetzung umfaßt, auf der das Färbemittel aus der Gasphase abgeschieden ist.

7. Verfahren nach Anspruch 1, wobei das Donorblatt einen Träger umfaßt, auf dem nacheinander eine, das Strahlung absorbierende Material umfassende, Strahlung absorbierende Schicht, gefolgt von einer Schicht des aus der Gasphase abgeschiedenen, thermisch übertragbaren Färbemittels, abgeschieden sind.

8. Verfahren nach einem der vorstehenden Ansprüche, wobei die Färbemittelschicht als Film mit anisotroper Topographie aus der Gasphase abgeschieden ist.

9. Verfahren nach einem der Ansprüche 1 bis 4, 6 und 7, wobei das Strahlung absorbierende Materie ausgewählt ist aus: Ruß und anderen Pigmenten, Nickeldithiolan-Farbstoffkomplexen, Eisenkomplexen, Cyaninfarbstoffen, Merocyaninfarbstoffen, Oxyindolizinfarbstoffen, Inden-verbrückten Polymethinfarbstoffen, dreikernigen Cyaninfarbstoffen, Bis(aminoaryl)polymethinfarbstoffen, Tetraarylpolymethinfarbstoffen. Chalkogenpyrlo-arylidenfarbstoffen, Bis(chalkogenpyrylo)polymethinfarbstoffen, Phthalocyaninfarbstoffen, Squaryliumfarbstoffen, von Anthrachinonen und Naphthochinonen abgeleiteten Farbstoffen und Croconiumfarbstoffen.

10. Verfahren nach einem der vorstehenden Ansprüche, wobei das thermisch übertragbare Färbemittel ein Farbstoff oder ein Pigment ist.

11. Verfahren nach Anspruch 10, wobei das Färbemittel ein organisches Färbemittel oder ein anorganisches Pigment, ausgewählt aus Metallen, Metalloxiden und Gemischen davon, ist.

12. Verfahren nach einem der vorstehenden Ansprüche, wobei Schritt (b) ferner das in engen Kontakt Bringen einer photographischen Maske mit den in Kontakt befindlichen Donor- und Rezeptorblättern und das Belichten der Einheit durch die photographische Maske umfaßt, wobei die Belichtungsstrahlung in den durch transparente Bereiche der Maske definierten Flächen eine thermische Übertragung von Färbemittel vom Donorblatt auf das Rezeptorblatt bewirkt.

13. Verfahren nach Anspruch 12, wobei auf die zusammengefügte Einheit aus photographischer Maske und Donor- und Rezeptorblättern ein Druck von mindestens 10 g/mm² ausgeübt wird.

14. Verfahren nach Anspruch 12 oder Anspruch 13, wobei die in Kontakt befindlichen Donor- und Rezeptorblätter ein System darstellen, das ausreichend empfindlich ist, um eine Übertragung von Färbemittel bei Energieniveaus von weniger als 4 J/cm² zu bewirken.

15. Verfahren nach einem der vorstehenden Ansprüche, wobei die Scanning-Belichtungsquelle ein Laser oder eine Laserdiode ist.

16. Verfahren nach Anspruch 15, wobei der Laser eine Leistung von mindestens 5 mW besitzt.

17. Donorblatt zur thermischen Übertragung, umfassend die Aufeinanderfolge eines Trägers, einer Strahlung absorbierenden Schicht, umfassend einen Farbstoff oder eine Kombination aus einem Pigment und einem Bindemittel, und einer Schicht eines aus der Gasphase abgeschiedenen, thermisch übertragbaren Färbemittels.

18. Donorblatt zur thermischen Übertragung nach Anspruch 17, wobei das Strahlung absorbierende Material Strahlung einer Wellenlänge von 600 bis 1070 nm absorbiert.

19. Donorblatt zur thermischen Übertragung nach Anspruch 17 oder Anspruch 18, wobei die Strahlung absorbierende Schicht eine Schicht eines Bindemittels umfaßt, in dem das Strahlung absorbierende Material gelöst oder dispergiert ist.

20. Donorblatt zur thermischen Übertragung nach Anspruch 19, wobei das Bindemittel der Strahlung absorbierenden Schicht eine Glasübergangstemperatur (T_{g}) von mindestens 100°C besitzt.

21. Kombination aus einem Donorblatt zur thermischen Übertragung nach einem der Ansprüche 17 bis 20 und einem Rezeptor für das thermisch übertragbare Färbemittel.

22. Medium zur thermischen Übertragung, umfassend ein Donorblatt mit einer Donorschicht, die eine Schicht eines aus der Gasphase abgeschiedenen, thermisch übertragbaren Farbemittels umfaßt, und ein Rezeptorblatt für das thermisch übertragene Färbemittel, umfassend ein Strahlung absorbierendes Material.

## Revendications

1. Procédé de formation d'image par transfert thermique qui comprend les étapes suivantes :
(a) la mise en contact d'une feuille réceptrice et d'une feuille donneuse comportant une couche de donneur comprenant un colorant thermiquement transférable de telle sorte que la couche de donneur soit en contact intime avec la feuille réceptrice, une des feuilles donneuse et réceptrice comprenant une matière absorbante de rayonnement pouvant absorber un rayonnement d'une source d'exposition de telle sorte qu'une exposition selon un mode de formation d'une image des feuilles mises en contact provoque un chauffage dans les régions exposées, ce chauffage provoquant un transfert thermique de colorant de la feuille donneuse à la feuille réceptrice en vue de former une image, et
(b) l'exposition selon un mode de formation d'une image des feuilles mises en contact en utilisant une source d'exposition à balayage, caractérisé en ce que la couche de donneur comprend une couche d'un colorant déposé en phase vapeur.

2. Procédé suivant la revendication 1, dans lequel le récepteur comprend un support sur lequel est appliquée une couche de récepteur pour le colorant et la matière absorbante de rayonnement est présente soit dans la couche de récepteur soit dans une couche sous-jacente séparée à celle-ci.

3. Procédé suivant la revendication 2, dans lequel la couche de récepteur comprend une couche d'un liant contenant la matière absorbante de rayonnement dissoute ou dispersée.

4. Procédé suivant la revendication 2, dans lequel la feuille réceptrice comprend un support sur lequel sont successivement appliquées une couche absorbante de rayonnement comprenant la matière absorbante de rayonnement et, comme couche supérieure à celle-ci, la couche de récepteur.

5. Procédé suivant la revendication 1, dans lequel le colorant transférable thermiquement déposé en Phase vapeur peut absorber le rayonnement d'exposition de telle sorte qu'il se transférera sans aide lors de l'exposition de la feuille mise en contact.

6. Procédé suivant l'une quelconque des revendications précédentes, dans lequel la feuille donneuse comprend un support comportant une couche de séparation contrôlée sur laquelle le colorant est déposé en phase vapeur.

7. Procédé suivant la revendication 1, dans lequel la feuille donneuse comprend un support sur lequel sont appliquées successivement une couche absorbante de rayonnement comprenant la matière absorbante de rayonnement suivie d'une couche de colorant transférable thermiquement déposée en phase vapeur.

8. Procédé suivant l'une quelconque des revendications précédentes, dans lequel la couche de colorant est déposée en phase vapeur sous la forme d'un film de topographie anisotrope.

9. Procédé suivant l'une quelconque des revendications 1 à 4, 6 et 7, dans lequel la matière absorbante de rayonnement est choisie parmi le noir de carbone et d'autres pigments, les complexes de colorants de nickel-dithiolène, les complexes ferreux, les colorants de cyanine, les colorants de mérocyanine, les colorants d'oxyindolizine, les colorants de polyméthine à pont d'indène, les colorants de cyanine trinucléaire, les colorants de bis(aminoaryl)polyméthine, les colorants de tétraarylpolyméthine, les colorants de chalcogénopyrylo-arylidène, les colorants de bis(chalcogénopyrylo)polyméthine, les colorants de phtalocyanine, les colorants de squarylium, les colorants provenant d'anthraquinones et de naphtaquinones et les colorants de croconium.

10. Procédé suivant l'une quelconque des revendications précédentes, dans lequel la matière colorante transférable thermiquement est un colorant ou pigment.

11. Procédé suivant la revendication 10, dans lequel la matière colorante est un colorant organique ou un pigment inorganique choisi parmi les métaux, les oxydes métalliques et leurs mélanges.

12. Procédé suivant l'une quelconque des revendications précédentes, dans lequel l'étape (b) comprend de plus l'assemblage d'un masque photographique en contact intime avec les feuilles donneuse et réceptrice mises en contact et l'exposition de l'assemblage à travers le masque photographique, le rayonnement d'exposition effectuant le transfert thermique de colorant de la feuille donneuse à la feuille réceptrice dans des Zones définies par les régions transparentes du masque.

13. Procédé suivant la revendication 12, dans lequel une pression d'au moins 10g/mm² est appliquée à l'assemblage constitué du masque photographique et des feuilles donneuse et réceptrice.

14. Procédé suivant l'une ou l'autre des revendications 12 et 13, dans lequel les feuilles donneuse et réceptrice mises en contact constituent un système qui est suffisamment sensible pour effectuer le transfert de colorant à des niveaux d'énergie inférieurs à 4J/cm².

15. Procédé suivant l'une quelconque des revendications précédentes, dans lequel la source d'exposition à balayage est un laser ou une diode laser.

16. Procédé suivant la revendication 15, dans lequel le laser a une puissance d'au moins 5mW.

17. Feuille donneuse de transfert thermique comprenant successivement un support, une couche absorbante de rayonnement comprenant un colorant ou la combinaison d'un pigment et d'un liant et une couche d'un colorant transférable thermiquement déposé en phase vapeur.

18. Feuille donneuse de transfert thermique suivant la revendication 17, dans laquelle la matière absorbante de rayonnement absorbe le rayonnement ayant une longueur d'onde de 600 à 1070 nm.

19. Feuille donneuse de transfert thermique suivant l'une ou l'autre des revendications 17 et 18, dans laquelle la couche absorbante de rayonnement comprend une couche d'un liant contenant la matière absorbante de rayonnement dissoute ou dispersée.

20. Feuille donneuse de transfert thermique suivant la revendication 19, dans laquelle le liant de la couche absorbante de rayonnement a une température de transition vitreuse (T_{g}) d'au moins 100°C.

21. Combinaison d'une feuille donneuse de transfert thermique suivant l'une quelconque des revendications 17 à 20 et d'un récepteur pour le colorant transférable thermiquement précité.

22. Milieu de transfert thermique comprenant une feuille donneuse comportant une couche de donneur comprenant une couche d'un colorant transférable thermiquement déposé en phase vapeur et une feuille réceptrice pour le colorant transféré thermiquement comprenant une matière absorbante de rayonnement.
